

March 15, 1960

H. I. SILVERSHER

2,928,948

LAMINAR RAY RESISTANT MATERIALS

Filed May 23, 1955

*FIG. 1.*



*FIG. 2.*



*FIG. 3.*



*FIG. 4.*



INVENTOR.

*HERMAN I. SILVERSHER*

BY *Harbin White*

ATTORNEY.

# United States Patent Office

2,928,948

Patented Mar. 15, 1960

1

2,928,948

## LAMINAR RAY RESISTANT MATERIALS

Herman I. Silversher, Los Angeles, Calif.

Application May 23, 1955, Serial No. 510,249

9 Claims. (Cl. 250—108)

This invention has to do generally with the shielding against harmful transmission of ray-like emanations of the type producable from fissionable materials. Primarily the invention is directed in certain of its aspects to improved compositions or combinations of materials for preventing or reducing neutron transmission, or the effects of neutron penetration, and in other and more particular respects, the invention deals with materials and material combinations having for their objective to shield against the transmission of both ray (alpha, beta and gamma ray) as well as neutron transmission.

Speaking first in terms of the last-mentioned objective, the invention contemplates shielding against or minimizing the effects of ray-type radiation by the use of multiple layer or laminated materials, which may employ different metal and resinous plastic materials, all as more particularly dealt with in my copending application Ser. No. 492,486, filed March 7, 1955, now U.S. Patent No. 2,858,451 issued October 28, 1958, on "Laminar Ray Shielding Materials," together with a material or mixture of materials resistive to neutron transmission, so that the entire composite or combination becomes protective against both ray and neutron transmission or radiation. Before entering into a description of the entire combination or composite, reference preliminarily may be had to those general contemplations of the invention which pertain particularly to the absorption or slowing down of neutron energy.

It is found that certain metals and their compounds serve effectively to produce absorption or slowing down of neutrons of varying kinetic energy produced by the bombardment of direct and secondary radiation. The particular metals contemplated are of the class consisting of boron, cadmium, and lithium. It appears that the effectiveness of any of these metals, whether in elemental or chemically combined form, is due to the presence and distribution of boron, cadmium, or lithium atoms, or mixtures thereof, across the path of the neutron flow to be de-energized. And it will be understood that such distribution of the metal atoms can be present whether the metal be used in elemental form or in chemically combined form. Where it is desired to use the metal chemically combined, generally speaking any of its compounds may be employed, notably inorganic compounds of the metal, including oxides, salts such as the chlorides, sulfates, nitrates, including salts complexed with other metals, and also acids and bases of the metals. Of the named metals, boron and its compounds are preferred, and accordingly in the description to follow reference will be had to the use of boron or its compounds as preferred, though typical of the class. And in further reference to boron, it is found advantageous for many purposes to employ boron in the form of boric acid because of the supplementary beneficial effects upon neutron absorption contributed by the hydrogen atoms in the acid.

The general effect created by the presence of boron or its compounds in a shield form or composition appears to be that neutrons of high kinetic energy will

2

react with the metal molecules, as well as with hydrogen present therein, and will tend to reach a state of thermal equilibrium and to be less likely to ionize or otherwise contaminate the material bombarded. As previously indicated, a shield so composed normally will be employed with a material or combination of materials used for shielding against alpha, beta and gamma ray transmission or radiation, since in most instances the nature of the total radiation will be inclusive of neutron effects as well as the named rays.

Generally speaking, the invention contemplates incorporating the boron or its compounds in or on a suitable carrier, for which any of various plastics, inclusive of thermo-setting resins, are eminently suited by reason of desirable shielding properties possessed by the resins themselves. Typical plastic resins are the polyethylene, urea formaldehyde, melamine, phenolic, vinyl, and epoxy-type thermo-setting resins. As illustrative forms or conditions in which the boron or its compounds may be applied to or incorporated in a carrier resin, reference may be had to the following: The neutron absorptive metal may be plated or coated on the plastic, as by plating a carbon or graphite loaded polyethylene plastic with cadmium. A suitable carrier or lamination, preferably 25 of resinous composition, may be coated with the metal or its compound (e.g. boric acid) by admixture with a fluid resin so that the admixture may be applied as a paint or caulking material. In laminated forms the metal or its compound, again typically boric acid, may be dispersed in an epoxy or other appropriate thermo-setting resin and the resulting compound used to laminate metals or fibers together, as disclosed in my prior application referred to above. Another practice may be to incorporate the metal or its compound in a plastic or wax, such 30 as polyethylene or paraffin, by physically mixing or milling, and then applying the composite as a film, layer or lamination, as the circumstances may require.

Where admixed with a resinous, waxy or other carrier or binder, the percentage of boron or its compounds may 40 vary depending upon any of various considerations such as the thickness of the shield, layer or lamination, and the degree of neutron shielding required. In general the proportion of metal or its compound may range as high as 50%, and to even higher levels so long as the quantity 45 and properties of the selected resin or other binder are sufficient to integrate the metallic additive in a continuous and ordinarily self-supporting mass. In most instances strength, hardness and rigidity will be imparted to the composite by curing of a thermo-setting resin binder 50 which, if desired, may be reinforced by pigment or filler or by glass fabric or fibers.

Referring now to the ray shielding materials or combinations thereof in conjunction with which the above-mentioned neutron absorptive materials may be used, it 55 is found that by reason of their relatively great density, certain metals of the group consisting of lead, uranium, thorium and thallium have a capacity to block ray transmission to a considerable extent by virtue of absorption of the rays. For purposes of further description, lead 60 may be regarded as typical and preferred because of its availability and cost advantages of metals in this class. The completeness of ray blocking by any of these metals, will be dependent upon the nature and concentration of the rays, as well as the total thickness of the metal barrier in any particular instance. It will be understood 65 that for the purposes of the invention, I may use one or more sheets of any of these metals, or combinations thereof, and which may range in thickness from about  $\frac{1}{1000}$  inch to 6 inches. Blocking of the rays by these heavier metals occurs at least partially by absorption in them of some of the ray energy, and gives rise to another phenomena in the nature of a secondary radiation.

of absorbed energy from the metal. As will appear, in dealing with the problem of preventing or limiting ray transmission, the invention also aims to reduce and minimize the secondary radiation effects.

The present composite material also employs the use of one or more sheets whose thicknesses may fall in about the same range of the thicknesses of the heavy metal, of one or more of such metals as copper, aluminum, brass, lithium, and ductile ferrous metals, whose effect upon the rays striking them is more in the nature of deflection or reflection, as distinguished from blocking by absorption and relatively low reflection. Aluminum may be regarded as illustrative of the metals in this second group. Thus in a composite employing for example lead and aluminum sheets, the aluminum serves to reduce by deflection or reflection of the rays, the ray energy and concentration to which the lead is subjected, and the aluminum serves further to reduce secondary ray emanations from the lead. The aluminum has a comparatively short half-life, i.e. the time during which it will continue to emanate previously absorbed rays.

It is preferred to further increase the ray blocking capacity of the composite and prevent or minimize neutron transmission by including therein one or more sheets of a polymerized resin or plastic material, which generally speaking may be selected from any of the so-called plastics capable of conforming to such deformation as the composite is to be given in any particular molding or shaping operation. Typically, the preformed plastic sheet or sheets, in thicknesses within the metal sheet thickness range, may be selected from such resins as polyethylene, fluorinated ethylenes, polystyrene and polybutene. Thus when so composed, all the laminations, metal and resin, have such ductility as will permit them to be shaped and deformed as desired.

The laminations are bonded together by the use of any suitable thermo setting resin which will cure at the temperature, which may range for example from about 100° F. to 350° F., at which the laminations are pressed together for integration and such shaping or deformation as may be required. Suitable bonding agents are the so-called B-stage (incompletely polymerized) resins of the additional type including the styrene base polyesters, epoxy resins and silicone resins, rubbers, and phenol formaldehyde resins. Among these the epoxy resins are often preferred because of such qualities as superior adhesiveness, flexibility and dimensional stability. The epoxide resins have the general formula:



wherein "R" represents the divalent radical of dihydric phenol and "n" is from 0 to 4. One major difference between various resins having this generic formula is in the (n) value which determines the length of the molecule. The more fluid the resin the smaller the (n) value. Generally these epoxy resins having a value for (n) of 2 or more are solid or essentially solid and may require solvent thinning for their use, whereas those having an (n) value of 0 or 1 are essentially stable fluids. It is these latter fluid epoxy resins which I prefer to use for the purposes of the present invention by reason of the facility possessed by the fluid resin for wetting the lead or lead silicate particles, and the resultant capacity of the resin to permit incorporation therewith of higher amounts of the lead or lead silicate in dense and uniform distribution. Accordingly, the preferred epoxy resins are those which are normally fluid, having an (n) value of from 0 to 1, and an epoxide equivalent between 140 and 550, the epoxide equivalent being defined as the grams of resin containing 1 gram equivalent of the epoxide group—



The epoxide resin is cured by cross linkage or addition polymerization with any of various compounds having amino or amide groups. Among the various amino or amide materials useable for the curing of epoxy resins are (2,4,6-tri(dimethylaminomethyl) phenol, diethylenetriamine, dimethyl amino propylamine, metal phenylene diamine, dicyandiamide, piperidine, and pyridine.

For certain purposes it may be desirable to favor the resiliency and toughness of the composite material by incorporating therein a plasticizer, for which purpose the polyamide resins have been found to be particularly satisfactory. These are resins having molecular weights ranging from 3,000 to 10,000, and are prepared by the condensation of polymerized unsaturated fatty acid (e.g. dilinoleic acid) with aliphatic amines such as ethylene diamine. Structurally, such polyamide resins have the formula



wherein "n" may range from 5 to 15. Typical of such resins is "Polyamide Resin 115" as sold by General Mills, Inc. In the case of the amino reaction, if the amine molecule contains more than one amino group, two or more epoxide units may be coupled together.

Relative to the curing effects and reactions of the amino group materials with relation to the epoxy resin, if the amine molecule contains more than one amino group, two or more epoxide units may be coupled together. The optimum amount of curing will occur when the epoxide and amino groups react, without any of either being left in excess after the reaction is completed. Thus the proper amount of any amino or amide group material to be used in the curing of the epoxy resin may be determined on a stoichiometric basis. In general the amide or amino group additive will range between from  $\frac{1}{20}$  to  $\frac{1}{2}$  weight parts to 1 part of the epoxy resin.

Where desired for additional strength and possible shear resistance in the bonding resin, the latter may be reinforced with such inert materials as glass or glass fibers or fabrics.

The invention contemplates further the incorporation of any of the aforementioned metals, heavy salts (e.g. lead monosilicate) and oxides thereof, or mixtures thereof, in any of the resinous components of the composite material. Thus the bonding agent, e.g. epoxy resin, may be admixed with up to around 15 weight parts of any of these metals, e.g. lead or aluminum, in powdered form, to improve the ray blocking or deflecting qualities



of the resin as such. Also the preformed sheet plastic material, e.g. polyethylene, may be composed of the resin containing uniformly distributed therein any of the powdered metals in whatever concentration desired so long as they are adequately integrated by the resin.

The invention will be further understood by reference to the accompanying drawing wherein I have shown certain typical and illustrative combinations of the sheet materials in interbonded laminar form. In the drawing:

Fig. 1 is a fragmentary section taken through a laminated composite containing two dissimilar metal sheets bonded together in direct relation;

Fig. 2 is a similar view showing the metal sheets indirectly bonded together by way of an intermediate resin sheet;

Fig. 3 is another view showing the metal sheets to be apertured where desirable for effecting stronger bonds; and

Fig. 4 is a view showing a simpler laminated composite embodying the invention.

In Fig. 1 the composite material is shown to include a sheet 10 of relatively dense metal, such as lead, bonded

to a sheet 11 of a deflective metal such as aluminum which in use, may be positioned between sheet 10 and the ray source. The two metal sheets are bonded together by a layer or common coating of a thermo setting bonding plastic 12, such as the epoxy resin which polymerizes as the composite assembly is heated and subjected to whatever pressure desired to urge the sheets together. Ordinarily it is preferred to include also a preformed plastic sheet 13, such as polyethylene, which may surface the composite at one or both sides of the metal sheets 10 and 11. The plastic sheet is bonded thereto at 14 using the same resin employed for bonding the metal sheets together or by mechanical attachment.

In Fig. 2 the lead 15 and aluminum 16 sheets are shown to be indirectly bonded to an inner positioned plastic sheet 17 by the bonding resin indicated at 18. As before, one or both metal sheets may be covered at the outside by plastic sheets 19.

Fig. 3 shows the metal sheets 20 and 21 to contain recesses or holes 22 wherever desirable to form a stronger bond, as with the plastic sheets 23 and 24. Here the bonding resin 25 may contain any of the metals, for example lead or aluminum, in powdered form, uniformly dispersed throughout the resin, for the purpose of minimizing ray transmission through the recesses or openings.

To cite a specific example of the invention in reference to Fig. 2, lead sheet 15, aluminum sheet 16 and plastic sheets 19 each may be around  $\frac{1}{8}$  inch in thickness, and are bonded together by polymerization of about 100 parts of an epoxy resin (e.g. Shell "Epon 828") and about 15 parts of meta phenylene diamine. The laminations are placed together as illustrated in a heated press or mold, and the resin cured at a temperature of about 280° F. A post cure at 350° F. will give optimum physical and structural properties.

The described embodiments of the invention in Figs. 1 to 3, may be supplemented for the purposes of neutron absorption, in any of various manners. For example, in Fig. 1 any or all of the epoxy resin laminations 12 and 14, and any or all of the laminations 18 in Fig. 2, and any or all of the laminations 25 in Fig. 3, may be supplemented by incorporating in the resin up to 50% or more of boron or boron compound, preferably boric acid, which may be uniformly distributed in finely divided form by admixture with the resin in an uncured state. The specific example given above pertaining to Fig. 2, is to be construed accordingly. Alternately, or in addition, the neutron absorptive metal or its compounds, may be similarly incorporated in either or both the surface layers 13 of Fig. 1, 19 of Fig. 2, and 24 of Fig. 3.

In Fig. 4, I show a further variational form of the invention in which bonded to a lead sheet 26 is a resinous lamination 27, composed typically of a thermally cured epoxy resin. Dispersed in the latter may be any of the neutron absorptive metals or their compounds, as previously described. Fig. 4 is illustrative of the further possibility of surface coating a layer or sheet, or layer composite, with uniformly distributed atoms of the neutron absorptive metal, whether in the elemental state or chemically combined. Thus, for example, to the resin layer 27 may be applied a coating 28 which for example may be cadmium electroplated on a resin lamination 27 rendered conductive by loading with carbon

and graphite, or the coating 28 may be applied in the form of a paint composed essentially of neutron absorptive atoms, typically as cadmium, boron or boric acid, in a resinous binder which may be thermally cured to hardness.

I claim:

1. An integrated laminous shielding material comprising a first layer of ray-blocking metal of the group consisting of lead, uranium, thorium and thallium, and a second layer comprising an organic resin carrying a uniformly distributed neutron absorbent of the group consisting of boron, cadmium and an inorganic compound of boron, cadmium and lithium.

2. A shielding material as defined by claim 1, in which said resin is a thermally hardened thermosetting resin.

3. A shielding material as defined by claim 1, in which said first layer is lead and said resin is a thermally hardened thermosetting resin bonded thereto.

4. A shielding material as defined by claim 1, in which said neutron absorbent is an inorganic compound of boron bonded to the first layer by said resin.

5. For use in ray shielding, the combination comprising a first layer of ray-blocking material of the group consisting of lead, uranium, thorium and thallium, a second layer of ray reflective metal of the group consisting of copper, aluminum, brass and ductile ferrous metals, a neutron absorbent of the group consisting of boron, cadmium and lithium uniformly distributed coextensively with common areas of said first and second layers, and an organic resinous carrier for said absorbent.

6. The combination as defined in claim 5, in which said resinous carrier is a heat hardened thermosetting resin.

7. The combination as defined in claim 5, in which said absorbent is uniformly distributed in a third layer comprising a thermosetting resin and said first layer is lead.

8. For use in ray shielding, an integrated laminar combination comprising a first layer of ray-blocking material of the group consisting of lead, uranium, thorium and thallium, a second layer of ray reflective metal of the group consisting of copper, aluminum, brass and ductile ferrous metals, and a third intermediate layer comprising a thermosetting resin containing a uniformly distributed inorganic compound of boron.

9. For use in ray shielding, an integrated laminate comprising a first layer of lead, a second layer of aluminum, and a third intermediate layer bonded to said first and second layers and comprising a thermosetting resin containing a uniformly distributed inorganic compound of boron.

#### References Cited in the file of this patent

#### UNITED STATES PATENTS

|    |           |              |                |
|----|-----------|--------------|----------------|
| 55 | 2,003,752 | Landt        | June 4, 1935   |
|    | 2,206,634 | Fermi et al. | July 2, 1940   |
|    | 2,522,522 | Krasnow      | Sept. 19, 1950 |
|    | 2,528,235 | Loritsch     | Oct. 31, 1950  |
|    | 2,580,360 | Morrison     | Dec. 25, 1951  |
| 60 | 2,727,996 | Rockwell     | Dec. 20, 1955  |
|    | 2,796,411 | Zirkle       | June 18, 1957  |
|    | 2,796,529 | Morrison     | June 18, 1957  |
|    | 2,807,727 | Fermi et al. | Sept. 24, 1957 |